

May 20, 1930.

D. H. YOUNG

1,759,561

KNITTED FABRIC

Filed Jan. 9, 1930

Fig. 1.



Fig. 2.



Fig. 3.



Fig. 4.



INVENTOR  
DAVID H. YOUNG

by his attorneys  
Howson and Howson

## UNITED STATES PATENT OFFICE

DAVID H. YOUNG, OF DALTON, GEORGIA, ASSIGNOR TO WESTCOTT HOSIERY MILLS, OF DALTON, GEORGIA, A CORPORATION OF GEORGIA

## KNITTED FABRIC

Application filed January 9, 1930. Serial No. 419,611.

This invention relates to knitted fabrics and more particularly to the nature of the yarn used. The invention will be described with relation to stockings but it is applicable 5 to stockings, underwear and other knitted fabrics. One of the disadvantages of stockings, especially those made of silk or rayon, is their luster, lack of opacity and their liability to start runs. These stockings are made 10 of yarns having a low twist of say three to eight turns per inch. I have discovered that a countertwisted yarn of any lustrous material with a high twist (within a certain range) of both the threads and the yarn, will 15 give a much more desirable article than the ordinary stocking. Where in the claim I speak of lustrous yarns I mean silk and synthetic yarns. The former lacks the usual luster, is more transparent, dyes better and 20 is stronger, more resistive to picking runs, capable of stretching more than stockings heretofore made, has a more uniform appearance and is not sleazy.

In the drawings Fig. 1 is a diagram of 25 a piece of fabric shown as made partly from ordinary single low twist yarn and partly from the new high countertwist yarn;

Fig. 2 is an enlarged diagrammatic view 30 of a piece of the new yarn;

Fig. 3 is a cross section diagrammatic of the yarn taken on the line 3—3 of Fig. 2; while

Fig. 4 is an outline of part of one type of stocking such as is knit from the new yarn.

Referring to the drawings, the part A of Fig. 1 shows ordinary fabric, and the part B shows my new fabric.

The novel yarn 5 which is used in the new stocking is prepared in the following manner. 40 Each individual strand or thread 6 is first wound in the usual manner and then spun. During this spinning it is preferable to give each individual thread 28 to 48 turns per inch, for example, but it will be obvious that these 45 limits are somewhat elastic. This twist may be put in pairs of threads rather than individual threads, i. e. it is in the first time spinning that it is put in. Where in the claim I speak of individual threads I refer 50 to the filaments which are twisted in the first

time spinning, whether individual threads or pairs. Twists of less than 28 turns per inch do not give much of the desired effects. After spinning the individual strands 6 they are doubled, i. e. put together. In the example 55 given the yarn 5 is a four thread yarn and the individual threads were each given 32 turns per inch to the left. After doubling, the yarn is spun again. This spinning is given in a direction opposite to the twist of the individual threads, i. e. to the right. I prefer to make the yarn twist from 28 to 44 turns per inch. Here again the limits are elastic. In the example shown in the drawings the yarn is given a twist of 28 turns per inch. The yarn is then coned as usual and it is ready for the knitting machine. It will be observed that by giving this high countertwist the width and cross sectional area of the yarn have been reduced, the yarn has been 70 made circular in cross section and a stiffer and stronger yarn produced. (See Fig. 3). I have found that the fewer the individual threads in the yarn the higher the twist required in both threads and yarn. 75

The yarn is fed to the needles in the knitting machine in the usual manner. The fabric resulting from the use of this novel knitting yarn has many admirable characteristics. In the first place the reduced surface of the 80 yarn and the fact that same is wound together with opposed twists of the yarn eliminates, to a great extent, the luster commonly found in silk stockings. The lines of the wales are less apparent to the naked eye than is the 85 case with the ordinary stocking and the fabric is more uniform and flatter. Also the fabric is much more transparent. In addition, the yarn can be stretched about a half more than stockings knit of ordinary yarn. This greater elongation is, of course, a tremendous advantage, especially in a seamless stocking. Furthermore, the greater shrinkage of the 90 yarn in manufacture gives it a uniform elasticity which automatically controls the sizes of the stockings making a more uniform product and one which fits a wider range of limbs. It has also been found that the nature of the yarn seems to be such that the "feel" 95 of the fabric is much more pleasant than in 100

the ordinary stocking. The stocking is less liable to start a run and has better dyeing qualities. Water spots are not so prominent on stockings made from my new yarn.

5 Modifications will doubtless occur to those skilled in the art which do not depart from my invention.

What I claim is—

- 10 1. A knitted fabric composed of a lustrous yarn having a plurality of individual threads, said threads having been given a twist in one direction and the final yarn a twist in the opposite direction, the twists given being of the order of 28 to 48 turns per inch.
- 15 2. A knitted fabric composed of a lustrous yarn having a plurality of individual threads, the individual threads having been given a twist in one direction in the first time spinning and the final yarn having been given a lower twist in the opposite direction, said twists having been of the order of 28 to 48 turns per inch and high enough to make the yarn substantially circular in the cross section.
- 20 25 3. A knitted stocking containing a silk yarn composed of a plurality of threads, each thread having been given a twist in one direction in the first time spinning and the final yarn having been given a lower twist in the opposite direction, said individual threads having been given a twist of the order of 32 to 48 turns per inch and said yarn a twist of the order of 28 to 44 turns per inch.
- 30 35 4. A knitted stocking containing a silk yarn composed of a plurality of threads, each thread being twisted in one direction and the yarn as a whole being twisted in the opposite direction, the twists given said threads and yarn having been twists of at least the order of 28 turns to the inch.
- 40 45 5. A seamless knitted stocking containing a silk yarn composed of a plurality of threads, each thread having been twisted 32 or more turns to the inch in one direction, and the yarn having been twisted in the opposite direction a lesser number of turns per inch but at least 28.
- 50 55 6. A seamless knitted stocking containing a silk yarn composed of a plurality of threads each having been twisted to the left 28 or more turns per inch, and the yarn having been twisted to the right a lesser number of turns per inch.
- 60 65 7. A knitted fabric composed of a lustrous yarn of a plurality of individual threads, said individual threads having been given a twist of the order of 32 to 48 turns per inch in the first time spinning and the final yarn having been given a twist of the order of 28 to 44 turns per inch in the yarn, the latter twist being opposite to the first.

In testimony whereof I have signed my name to this specification.